

## UNITED STATES PATENT OFFICE

2,001,427

## ART OF COLORING ALUMINUM ARTICLES

James Francis Leahy, Fairhaven, Mass., assignor  
to Atlas Tack Corporation, Fairhaven, Mass., a  
corporation of New York

No Drawing. Application May 14, 1930,  
Serial No. 452,525

11 Claims. (Cl. 148—6)

This invention relates to the art of coloring aluminum or aluminum alloys, being more particularly applicable to fabricated, small aluminum articles such as buttons, eyelets, and the like. An object is to make possible a more economical, uniform, and durable coloring of such articles than that effected by the use of so-called japans, varnishes, and lacquers. Another object is to make possible the handling of a large number of such articles in a batch without requiring any particular arrangement of the articles, thereby obviating the trouble and expense incident to the handling of the individual articles.

I have found that if such articles are superficially oxidized and are then treated with mordant dyes, insoluble color lakes may be tenaciously fixed in situ on the aluminum base in sufficiently hard and dense condition that they are resistant to the abrasion of handling or use. The reaction is evidently analogous to that occurring when textile goods are treated with mordant dyes, as in such case aluminum oxide or other metallic oxides are used to fix the dye on the goods.

The superficial oxidation of aluminum may be effected in a great many ways, but I have found that solutions of oxidizing agents, and more specifically a solution of sodium carbonate and sodium bichromate, not only effect the desired reaction very quickly, but produce a dense, hard coating of oxide which is strongly adherent to the aluminum base. This oxide is a mixture of both aluminum and chromium oxides, the sodium bichromate evidently being reduced by the metallic aluminum into an oxide while serving to oxidize the metallic aluminum into an oxide. In order to effect a rapid and uniform coloration of the oxide-coated base, it is distinctly desirable and in most cases necessary to use an acid solution of the dye, but only weak or slightly ionized acids have been found satisfactory for this purpose.

Various specific examples of procedure falling within the purview of the present invention are possible, but I shall give one example which has been found to give eminently satisfactory results on a commercial scale. Aluminum articles, such as buttons, are placed in a suitable perforated container or basket, and the basket then immersed in a solution of about 2% sodium carbonate and about 1/2% sodium bichromate, preferably at boiling temperature, as elevated temperature serves to accelerate the reaction. The articles need remain in contact with the boiling solution for only about five to fifteen minutes, at

the end of which time a coating or skin of oxide of the desired depth has been produced and little further reaction takes place, probably owing to the impermeable character of the coating. The basket of articles is then removed from the solution and is preferably washed free of entrained solution, as by dipping into a bath of wash water. It is then immersed in a bath, preferably at about boiling temperature, containing about 1% of a lake-forming or mordant dye, of the desired color, for instance alizarin red, blue, or green, or a mixture of such dyes, and about 1% of a weakly ionized acid, such as formic, acetic, lactic, tartaric, boric, or phosphoric, and the articles permitted to remain in contact with the dye for about fifteen minutes, at the end of which time a practically maximum coloration has been effected. The use of a dye bath at elevated temperature is highly desirable, in that the reaction to form the colored coating is greatly accelerated by increase of temperature, little reaction taking place at room temperature. The articles may then be dried; and, if desired, this may be effected in a current of warm air, inasmuch as no visible discoloration takes place under such conditions. The insoluble color lake formed on the articles is resistant to scratching or abrasion, and is characterized by its density, hardness, and tenacity. It is firmly bonded with the aluminum base, but it can be removed by a hard, sharp instrument. The color lake resists removal, even by repeated treatment in solutions of alkali or soap such as are used for laundering purposes, so that aluminum buttons colored in accordance with my process are especially suitable for use on shirts or other articles of apparel which undergo repeated laundering treatment. This resistance to removal of the dyed coating by washing fluids is in marked contrast to the ready removability of the uncolored oxide coating by the same agents. It has been found necessary for the purpose of developing the desired colored or dyed coating to treat the articles with the dye solution while the coating of oxide is in a wet and comparatively freshly formed condition as a result of the treatment with the oxidizing solution. The superficially oxidized articles should hence not be dried or be kept much longer than a day, even if maintained under water, for, if they are once dried or allowed to stand for, say, a week, even under water, there is little or no color reaction when they are treated with the dye solution. This characteristic of the coating is of advantage in that a dry- 55

ing step between the treatment with an oxidizing solution and a dye solution is avoided.

In addition to those advantages already enumerated, my process possesses merit in that it 5 may be practised with inexpensive apparatus and with little consumption of chemical or dye. The oxidizing and dye baths which I employ may be reused many times, with the addition of such little make-up chemical or dye as has been removed by reaction on the aluminum articles or 10 by entrainment. Another advantage of my process is that it makes possible the use of a family of organic dyes which includes a large variety of colors or tints. While I cannot state with 15 precision what reactions take place in the oxidizing bath, nevertheless it appears probable that the sodium carbonate converts the metallic aluminum into the oxide and that the sodium bichromate favors reaction and is itself reduced 20 in such a way as to produce an oxide coating having the desired physical characteristics. The part played by the acid in the dye baths has not been ascertained, but it may perform the function of a catalyst, perhaps initially reacting 25 with the aluminum oxide to form salts, which, in turn, react with and fix the dye in the desired insoluble condition.

I claim:

1. A process of coloring aluminum articles, 30 which comprises treating such articles with a solution of sodium carbonate and sodium bichromate to form a coating of aluminum and chromium oxides, and, while the coating is wet and in freshly formed condition, treating it with 35 a solution of a lake-forming dye containing added weakly ionized acid to form an insoluble color lake on such articles.

2. A process of coloring aluminum articles, 40 which comprises immersing such articles in a hot solution of about 2% sodium carbonate and about 1/2% sodium bichromate to form a coating of aluminum and chromium oxides, and then immersing the coated articles in a hot solution of about 1% of a lake-forming dye and 1% of 45 a weakly ionized acid to form an insoluble color lake on such articles.

3. A superficially colored article, comprising

an aluminum base coated with an insoluble color lake consisting of the reaction product of mixed aluminum and chromium oxides with a lake-forming dye solution containing added slightly ionized acid.

4. A process of coloring aluminum articles, 5 which comprises treating such articles with a solution of oxidizing agents, and thereafter subjecting the coated articles to the action of a mordant consisting of a weakly ionized acid and 10 of a lake-forming dye.

5. A process of coloring oxide-coated aluminum, which comprises treating the oxide-coated surface with a dye solution containing a weakly 15 ionized acid.

6. The method of coloring oxide-coated aluminum, which comprises treating the oxide-coated surface with a dye solution containing acetic acid.

7. In a process of coloring aluminum articles, 20 those steps which comprise treating the articles with a solution of an oxidizing agent to form a coating of oxide on the articles, and immediately thereafter treating the freshly coated articles with a dye solution containing a weakly ionized 25 acid.

8. A superficially colored article, comprising an aluminum base coated with an insoluble color lake comprising the reaction product of aluminum oxide with a lake-forming dye solution containing added slightly ionized acid.

9. A superficially colored article, comprising an aluminum base coated with an insoluble color lake comprising the reaction product of aluminum oxide with a lake-forming dye solution containing added acetic acid.

10. A process of coloring oxide-coated aluminum, which comprises treating the oxide-coated surface in the presence of weakly ionized acid 40 with a dye solution.

11. A superficially colored article, comprising an aluminum base coated with an insoluble color lake comprising the reaction product of aluminum oxide in the presence of weakly ionized acid 45 with a dye solution.

JAMES F. LEAHY.